

## UNITED STATES PATENT OFFICE.

LEONARD SHIPLEY, OF DUNDALK, MARYLAND, ASSIGNOR TO AMERICAN SMELTING AND REFINING COMPANY, OF NEW YORK, N. Y., A CORPORATION OF NEW JERSEY.

## METHOD OF CASTING COPPER.

No Drawing.

Application filed June 20, 1924. Serial No. 721,191.

To all whom it may concern:

Be it known that I, LEONARD SHIPLEY, a citizen of the United States, and resident of Dundalk, in the county of Baltimore and

5 State of Maryland, have invented certain new and useful Improvements in Methods of Casting Copper, of which the following is a specification.

This invention relates to the casting of 10 copper in bars, ingots, slabs and various other shapes.

The slabs and other shapes cast according to present methods have always had a rough or irregular upper surface, full of 15 ridges and furroughs, so much so that the products in fact have been classified by the characteristic appearance of these ridges. Thus, if the ridges are close together, the 20 copper is said to be "close set" and "coarse set" if the ridges are further apart.

For certain purposes, such as the drawing of fine wire and rolling of thin copper sheets, this so-called "set" becomes objectionable, causing cracks and imperfections to run 25 through the finished product.

Another objectionable feature has been the so-called "pitch" of the upper surfaces of the cast ingots or slabs, these being classified as of "high pitch" if of a convex surface, "flat pitch" if level and "low pitch" if concave.

The objects of this invention are to overcome and eliminate these imperfections or irregularities and to produce a cast copper 35 product having a substantially smooth regular upper surface free of imperfections which might run through the subsequently formed products.

I have discovered that the objectionable 40 unevenness which has heretofore been characteristic of the copper castings is occasioned by the formation of a film of oxide on the top surface which forms a wavy or ridgelike structure as the metal contracts 45 and gives up absorbed gases under the cooling influence of the atmosphere.

These results are prevented in this invention by covering the molds immediately after the molten copper is poured and keeping 50 them covered until the copper sets.

In the present practice of the invention, the molten copper is poured from the ladle into the molds of the casting machine, as usual, and as soon as each mold is filled, 55 it is immediately covered to shut off access

of air and hence prevent oxidization of the surface. This immediate covering also prevents sudden degasification of the copper before it sets.

Asbestos or materials that are poor heat 60 conductors provide the best covers for the molds, but copper, iron, brick and stone have been found satisfactory as covers for delaying the cooling action and producing a smooth, flat top slab or casting.

The mold covers must not fit hermetically tight, but should be close enough to prevent direct contact of the atmosphere with the copper. A clearance of one-half inch or even more between the sides of the mold 70 and the cover is permissible in practice since it is desirable to allow speedy escape of the occluded gases.

After the copper sets, which requires from 75 about three to seven minutes, depending upon the thickness of the bar and various other factors, the cover is removed from the mold and the casting is cooled by water spray or otherwise treated in the usual manner.

By covering the copper immediately after 80 it is poured and while still in a molten condition, the formation of the heretofore characteristic rough surface of the casting presents as smooth a surface as the sides which lie in contact with the mold walls. A 85 superior product is thus produced, which can be drawn, rolled or otherwise treated with certainty of the results being uniform and free from imperfections.

The absence of the characteristic set or 90 pitch also makes the casting solid and of the same density throughout its dimensions. The appearance of the new slabs or castings also is better, making them more desirable and marketable products.

95 What is claimed is:

1. The method of casting copper shapes which comprises pouring the molten copper into open molds and immediately covering the molds closely enough to prevent free 100 contact of atmosphere while permitting escape of the occluded gases and during a time sufficient to prevent surface oxidization, rapid cooling and sudden degasification of the copper.

2. In the casting of copper in open molds, a step which includes covering the open molds containing the molten copper until the molten metal has set.

105 3. The method of producing cast copper 110

shapes with smooth top surfaces which includes the step of covering the molds immediately after pouring the molten metal thereinto closely enough to prevent free access of air thereto but allowing for escape of occluded gases and for a time sufficient for the molten metal to set.

4. The method of casting copper shapes with smooth top surfaces which comprises

pouring the molten metal in open molds, <sup>10</sup> covering the molds to prevent free access of air to the molten metal, uncovering the mold after the metal has set and then cooling the solidified shape.

Signed at Baltimore in the county of <sup>15</sup> Baltimore and State of Maryland this 6th day of June A. D. 1924.

LEONARD SHIPLEY.